

## UNITED STATES PATENT OFFICE

2,160,162

ADHERENT GREASE AND METHOD FOR  
MANUFACTURING THE SAME

Arnold J. Morway, Roselle, and John C. Zimmer,  
Hillside, N. J., assignors to Standard Oil De-  
velopment Company, a corporation of Dela-  
ware.

No Drawing. Application March 14, 1935,  
Serial No. 11,002

9 Claims. (Cl. 87—9)

The present invention relates to an improved grease composition which is characterized by strong adherent properties. The composition and its method of manufacture will be fully understood from the following description.

5 Adherent greases have been known to the prior art but those now available are not entirely satisfactory. This particular type of grease is characterized by the property of adhering so strongly 10 to metal parts that the grease is caused to permanently string out without separating from the metal parts. These greases are to be clearly distinguished from the buttery or elastic type greases which tend to separate rapidly from the metal 15 parts and ball up rather than permanently string out. The adherent greases do not tend to spatter under sudden shock as do the buttery type greases and for this reason the former are more desirable where there is a likelihood of sudden shock 20 or centrifugal force which tends to pull the grease away from the metal parts to be lubricated.

The former or known adherent greases have been usually prepared from lubricating oils and aluminum stearate or similar aluminum soaps, and rubber has been added, sometimes in the 25 form of latex. These materials are added to the oil, which is heated to incorporate the soap and drive off any water and to form the grease. Such a grease is useful but has certain undesirable properties; for example, it tends to lose its structure if water is present and very stable emulsions are formed which are, of course, highly objectionable. Also, this type grease tends to pull out 30 and leak excessively from the bearing. These difficulties with the present known grease are characteristic of the aluminum soap used in their composition and it is highly desirable to produce an adherent grease which will not have these 35 objectionable features.

40 It is proposed herein to prepare an adherent lime soap grease by the addition of rubber in the form of latex or otherwise in order to obtain the advantages of the lime soaps which make a grease more stable toward working and more re-  
45 sistant to the action of water and showing less loss by leakage than the aluminum soap com-  
pounds referred to above. It has been found, however, that the ordinary method of manufac-  
turing the aluminum soap greases, in which the 50 oil soap and latex are mixed together and gently heated to remove the bulk of the moisture, is not applicable to lime soap greases containing rubber. Lime soap products produced in that way are en-  
tirely unsatisfactory because they are heavy fluid 55 compounds devoid of all grease structure. The

reason for the difference in the behavior of lime and aluminum soap compounds is unknown and the present applicants content themselves with noting this difference and disclosing a suitable method of manufacturing an adherent lime soap grease containing rubber.

In the manufacture of the lime soap grease it has been found to be important to add the rubber to a formed lime soap grease, that is to say, to add the rubber to a primary lime soap mixture 10 which has a firm grease structure. If the rubber is added say to the oil or soap before the grease structure is obtained, it has been found that heavy fluid mixtures are produced which do not possess a grease structure. In this respect 15 the lime soap compounds differ from those containing aluminum soaps.

The oil used in the present invention is a lubricating oil and may be selected from any particular source, such as the paraffinic, mixed or naphthenic base crudes, and may be of any type, such as the distillate or residual oils, and viscosity ranges of say from 75 to 2000 seconds Saybolt 20 at 100° F. may be selected. However, it is possible to vary the proportion of the other ingredients 25 to use an oil from say 200 to 500 seconds at 100° F. for almost all grades of grease.

Lime soaps may be prepared from any of the ordinary soap stocks, for example, from animal fats such as tallow, horse fat and the like, or 30 from vegetable oils such as cottonseed or cocoanut oils and the like, or from fish oils or the fat or soap acids of commerce such as oleic or stearic or their admixtures, or from synthetic acids obtained by the oxidation of heavy oils and waxes 35 at low temperatures. The amount of the soap in the final composition depends to some extent upon the particular soap used and on the quality of the grease desired but in most instances from 3 or 4 to say 30% may be used as wide limits and 40 ordinarily from 5 to 15% is commercially most desirable.

Rubber is preferably added to the grease in the form of latex, a natural milky emulsion of rubber as it is obtained from the rubber tree, but rubber 45 solutions in benzol may be used or other artificial dispersions. The amount of rubber in the finished grease should not be over about 5% by weight in any case, and may be as low as .1% in some instances.

50 Other materials may be added to the composition, such as anti-oxidants to prevent the deterioration of the rubber, for example .001 to .1% of aldon alpha naphthylamine, or similar known aromatic amines or hydroxy compounds. Fillers

such as chalk or graphite may be added, or wax, petrolatum, lubricating oil dyes, glycerine, glycols, or the higher alcohols, to produce particular qualities desired for specific purposes. A small amount of water is almost always present as in all lime greases, say from  $\frac{1}{4}$  to 5% of the whole, in order to produce a smooth, uniform soap dispersion free from lumps.

In the manufacture of the grease a major portion of the oil is placed in a kettle and the fat or fat acid added thereto. This mixture is heated and lime, preferably hydrated lime, added with constant heating and agitation so as to effect the saponification and dehydration. Materials other than the rubber may be added at this point if desired and the mass is cooled say to about 200° F., at which point water may be added so as to have present the requisite amount and the soap dispersion formed. The mixture is then further cooled to say 100° F. or below, producing a firm grease structure. This product will be referred to herein as the primary grease.

The latex is added to a minor fraction of the oil and this is gently heated so as to drive off the water present in the latex, leaving the rubber particles dispersed throughout the oil. The amount of oil used for this purpose should be calculated so as to produce a dispersion containing not more than say 1 to 5 or 10% of rubber, as this is about as heavy as can be conveniently handled. This mass is completely dehydrated, preferably under vacuum or by blowing with air, and is then thoroughly stirred or worked into the primary grease at a temperature of say 100 or 150° F. until uniformity is attained.

As a specific example of the present grease mixture and its method of preparation, the following examples may be given:

#### Example I

An ordinary lime soap grease was prepared having the following composition:

|               | Percent |
|---------------|---------|
| Lime soap     | 12      |
| Solar Red oil | 86      |
| Glycerine     | 1       |
| Water         | 1       |

This grease was soft and buttery and had an A. S. T. M. penetration of 325 at 77° F. The grease was not adherent.

#### Example II

A lime soap compound was prepared of the following composition, using the same fatty materials and the same oil as in the previous example, but including rubber. The material was made by putting the fat, oil, lime and latex into a kettle and heating to 350° F., then agitating to remove the bulk of the water which was adjusted to 1%:

|               | Percent |
|---------------|---------|
| Lime soap     | 12.0    |
| Rubber        | 0.5     |
| Glycerine     | 1.0     |
| Water         | 1.0     |
| Solar Red oil | 85.5    |

This mixture did not have a grease structure but was a heavy fluid. The penetration was infinite, in other words, the cone dropped through the sample without meeting resistance such as a grease offers.

#### Example III

An adherent grease was then prepared according to the present method, having an ap-

proximate composition very close to that given in Example II but with a definite, firm grease structure. About 87% of the Solar Red oil was used to prepare the primary grease, which contained no rubber. The dispersion of rubber in oil was prepared with the balance of the oil, about 15%, and the latex. After dehydration, this rubber dispersion was thoroughly stirred into the grease at a temperature varying between about 70 and 100° F. in order to make the finished adherent grease. The actual composition was as follows:

|           | Percent |
|-----------|---------|
| Lime soap | 12.0    |
| Glycerine | 1.0     |
| Rubber    | .5      |
| Water     | .75     |
| Oil       | 85.75   |

This grease had an excellent structure, showed a penetration of 367 at 77° F., and was firm with stringy, adherent properties.

#### Example IV

The following comparative tests show the advantages of lime soap greases containing rubber over the ordinary buttery lime greases or the aluminum soap greases containing rubber. The samples are as follows:

- #1—a lime soap grease containing about 12% of the soap with no rubber.
- #2—an aluminum soap grease containing 0.5% rubber.
- #3—a grease similar to #1 to which has been added 0.5% rubber and made according to the present invention.

|    | A. S. T. M. penetration (sec.) |         |        |
|----|--------------------------------|---------|--------|
|    | @77° F.                        | @30° F. | @0° F. |
| #1 | 322                            | 265     | 198    |
| #2 | 376                            | 229     | 153    |
| #3 | 360                            | 248     | 210    |

It will be observed that #2 became excessively hard at 0° F. while #3 showed the least change.

The average delivery pressure required for greasing pin and bushing shackles with a Ball-Crank gun were observed with the three samples at 0° F.

|    | #/sq. in. |
|----|-----------|
| #1 | 1350      |
| #2 | 2200      |
| #3 | 1100      |

The pressure required in the case of #2 is twice that required for #3, indicating the much greater ease of servicing.

A well worn Chevrolet 1931 model was put under test with the three greases and the mileage at which squeaks were noticed was determined after each servicing.

|    | Miles |
|----|-------|
| #1 | 250   |
| #2 | 800   |
| #3 | 1200  |

The present invention is not limited to any theory of the grease for adherent properties nor to the particular composition given in the illustrative examples, nor to any particular method of manufacturing the grease, but only to the following claims in which it is desired to claim all novelty inherent in the invention.

We claim:

1. Method for preparing an adherent lime soap grease composition comprising thoroughly incorporating a lime soap into a lubricating oil while heating the mixture to form a rubber-free primary product having a substantially stable grease structure, forming a dispersion of rubber in an additional quantity of said lubricating oil, cooling the primary product, and incorporating 10 said dispersion of rubber in oil with said product at substantially the temperature thereof.
2. A method for preparing an adherent and coherent lubricating composition comprising, thoroughly incorporating a lime soap into a lubricating oil, while heating the mixture, cooling the mixture to obtain a primary product having a substantially stable grease structure and working into said product a small amount of rubber dispersed in a solvent therefor.
3. Method according to claim 2 in which the 20 water content of the primary mixture of the lime soap and the oil is adjusted to an amount less than 5%, and the mass is cooled to obtain a smooth grease structure before the addition of 25 the rubber dispersion.
4. Method according to claim 2 in which the rubber dispersion in oil contains less than about 5% of rubber.
5. A method according to claim 2 in which the mixture of lime soap and lubricating oil is prepared at a temperature about 200° F. and the dispersion of rubber in solvent worked into the primary product after cooling to a temperature between 70° and 150° F. 5
6. A method according to claim 2 in which the 10 ingredient rubber is uncoagulated rubber from latex.
7. A method according to claim 2 in which the 15 rubber is dispersed in a hydrocarbon solvent therefor.
8. A method according to claim 2 in which the rubber is dispersed in a lubricating oil as a solvent therefor.
9. A method according to claim 2 in which the 20 dispersion of rubber is dehydrated to a substantial degree prior to its incorporation in the primary product. 20

ARNOLD J. MORWAY.  
JOHN C. ZIMMER.